

Dec. 7, 1926.

1,609,785

C. J. STEEN ET AL

METHOD AND DIES FOR PRODUCING FORGED CIRCULAR DISKS

Filed Jan. 12. 1924

2 Sheets-Sheet 1

Fig. 1.



Fig. 2.



Dec. 7, 1926.

1,609,785

C. J. STEEN ET AL

METHOD AND DIES FOR PRODUCING FORGED CIRCULAR DISKS

Filed Jan. 12, 1924

2 Sheets-Sheet 2



## UNITED STATES PATENT OFFICE.

CHRISTIAN J. STEEN, OF PHILADELPHIA, PENNSYLVANIA, AND EDWARD V. FINERAN,  
OF SEASIDE HEIGHTS, NEW JERSEY.

## METHOD AND DIE FOR PRODUCING FORGED CIRCULAR DISKS.

Application filed January 12, 1924. Serial No. 685,796.

Our invention relates to a method of producing disk forgings such as blanks for bucket wheels of steam turbines and the like, and the dies used in connection therewith.

5 Ordinarily the blanks for the bucket wheels are obtained by pressing the billets into the desired shape between dies that have the contour of the wheels. Experience has shown, however, that no satisfactory results are obtained in this manner because the surfaces of the wheel blank become wavy or crinkled.

10 The present invention now aims to avoid this disadvantage and to produce a wheel blank that is homogeneous and has a plane and even surface when it leaves the forging press.

15 The special dies forming the subject matter of the present invention are consequently arranged tangentially above and below the forging in the press so that only a small rectangular area is treated for each stroke of the press plunger.

20 In the accompanying drawing, one embodiment of the invention is illustrated, and—

Figure 1 is a plan view of bottom dies and turntable as arranged on a forging press;

25 Figure 2 is an elevation, partly in section, of the dies and turntable in position on the press;

Figure 3 is a side elevation of the dies;

Figure 4 is a transverse section along line 4—4 of Figure 3;

30 Figure 5 is a top plan view of a blank showing the result of the pressing in accordance with the present invention;

Figure 6 is an end view of Figure 5, and—

35 Figure 7 is a similar view of a wheel blank produced by ordinary methods, and Fig. 8 is a fragmentary sectional view of some details.

40 In the drawings, reference numeral 10 represents a false bottom supported on the base 11 of a forging press and numeral 12 represents a false top bolted or secured in any suitable manner under the press head 13.

45 Centrally in the false bottom 10 is provided a lifting cylinder 14 in which is mounted to reciprocate axially a piston 15 terminating at its upper end with a crown 23. Upon this crown is mounted to revolve a turntable 16 between which and the crown 50

55 is preferably inserted an antifriction bear-

ing 17 such as a ball or roller bearing. The turntable has a number of upstanding horns or gripping fingers 18 intended to engage with the under side of the forging 19.

The turntable is adapted to be intermittently rotated between each stroke of the press head and this may be accomplished in any suitable manner as, for instance, by a pawl 20 carried on the under side of the turntable 16 and engaging ratchet teeth 21 on a wheel and gland 22 which is fixedly mounted upon the false bottom 10 around the piston 15. It is evident that the revolving of the turntable may be accomplished by other means.

70 The raising and lowering of the turntable is accomplished by hydraulic or other means for which purpose an inlet pipe 24 leads into the bottom of the lifting cylinder 14.

75 Each of the bottom dies 25 has a foot plate 26 provided with apertures for securing bolts 27 which in the usual manner engage with their heads in T-slots running transversely in the false bottom 10. From the foot plate 26 rises a straight ridge 28 having a downwardly sloping parallel sides 29 and a flat narrow top face 30. The length of the die is slightly greater than half the length of the false bottom 10.

80 At its centrally positioned end the ridge 28 has an inwardly projecting heel 31 the top face 32 of which slopes down gently from the top surface 30 of the ridge 28.

85 An arm 33 projects in longitudinal direction from the ridge 28 and terminates with an ear 34. In the body of the ridge 28 is furnished an aperture 36. Brace rods 35 connect the two bottom dies 25, each of the rods engaging an ear 34 of one die and an aperture 36 of the other die. The bars are 90 thus arranged parallel with and equidistant from the vertical diametrical plane running through the axis of the turntable 16 and sufficiently far apart to clear, at all times, not only the horns 18 of the turntable but also 95 the hub 37 of the bucket wheel 19 after it has been formed. The brace rods also serve for adjusting the distance between the dies to take care of various diameters of hubs.

100 The top dies 40 are in all respects like the bottom ones with the exception that only one brace rod 41 is used running through apertures 42 provided in the heels 43. This brace rod will consequently be situated in 105 the said diametrical vertical plane there be- 110

ing no obstructions in the way. No arms 33 need therefore be provided on the upper dies.

These dies are secured to the false top 12 in the same manner as the lower ones to the false bottom, namely by bolts 44, the heads of which engage in corresponding T-slots 45 in the false top. The latter is in the usual manner bolted to the head 13 of the 10 forging press, while the false bottom 10 is secured to the base 11.

In Fig. 7 is represented the result of the ordinary manner of producing a forged disk. The surface 46 of the blank is crinkled or 15 wavy.

The following are the steps in producing a disk or wheel blank or finished forging in accordance with the present invention:

First, from an ingot is cut a billet of the 20 proper weight for the finished forging and shaped under a forging-press or hammer into a round flat disk which in the following will be called the "cheese" and constitutes the preliminary forging. The disk should 25 be of approximately the same thickness as that of the wheel hub of the finished forging.

Second, with top and bottom dies secured to the top plate 12 and the bottom plate 10 as indicated in the drawings, and adjusted with the heels 31 diametrically opposite each other to the exact diameter of the hub of the finished forging; the "cheese" is now inserted between the stationary bottom dies 35 and the raised top dies and permitted to rest upon the fingers 18. The hydraulic pressure in the lifting cylinder has been previously applied so that the turntable 16 carries the "cheese" with its bottom face 30 slightly above the top faces 30 of the die 40 ridges 28 permitting the turntable to turn the "cheese" freely when the press head with the top dies is raised.

Third, the press head with the top dies 45 is now lowered against the "cheese", when the latter descends together with the lifting cylinder piston until meeting with the ridges and heels of the bottom dies 25. A narrow groove 50 or channel is thus produced by 50 each of the ridges on both sides of the "cheese" terminating at the inner end with an inclined surface running inwardly from said groove or channel in radial direction of the "cheese", this inclined surface 50 being produced by the sloping heel of each die. The squeezing of the metal thus takes place 55 tangentially of the wheel by the die ridges while the heels compress the metal inwardly in radial direction around the hub 37 instead of outwardly. The metal is thus 60 pressed into greater compactness.

Fourth, the press head is raised sufficiently to permit the top dies to leave the "cheese" and the latter will be slightly lifted from 65 the bottom dies by the pressure exerted in

the lifting cylinder against the piston 15. The pawl 20 shifts position from one tooth to another depending upon the setting of the adjuster screw against the bottom of the turntable 16. As the distance is increased between the crown 23 and the ratchet wheel 22, and the "cheese" is free from both top and bottom dies, the pawl 20 will take a nearly vertical position and thus the ratchet gear causes the revolving of the turntable with the "cheese" through a small angle due to the pawl on the downward stroke engaging another tooth 21 on the stationary wheel 22. In this manner other sections of the top and bottom surfaces of the "cheese" are exposed to the ridges and heels of the dies.

For each stroke of the press head a new channel or groove is thus produced by each die in the top and bottom surfaces of the "cheese" until after a complete revolution of the latter its surfaces will have the appearance indicated in Fig. 5 of the drawings.

The longer the process is continued and the more turns the "cheese" is permitted to make, the less pronounced will the channels or grooves be until finally a smooth surface is produced entirely devoid of a wavy or crinkled edge.

Another advantage in forging a wheel blank in this manner is the packing or building up of the metal around the hub, thus insuring a full forging, this being caused by the heel or hub-forming projection on the die.

As will now be understood the method simulates very closely hand forging of a wheel.

Having thus described the invention, what is claimed as new is:

1. A die for circular forgings, comprising a foot portion adapted to be secured in a forging apparatus and a two armed body-portion of uniform height and substantially L-shaped configuration forming a ridge rising from the foot portion and having upwardly converging side and end surfaces, one of said arms being arranged radially and the other arm arranged tangentially with regard to the forging, whereby the radial arm is adapted to form the hub and the tangential arm the remainder of the forging, substantially as described.

2. A die for circular forgings, comprising a foot portion adapted to be adjustably secured in a forging apparatus and a ridge portion of substantially uniform height rising from the foot portion and consisting of a short arm arranged radially and a long arm arranged tangentially with regard to the circular forging, and the top surface of the short arm sloping downwardly from the top surface of the long arm in order to form a hub portion on the circular forging, substantially as described.

3. The combination with a forging press having a stationary member and a reciprocating member; of dies adapted to be adjustably secured to said members respectively, 5 each of said dies comprising a foot, a ridge rising from said foot and having a substantially rectangular top surface and downwardly diverging side faces, and a side projection extending substantially at right angles from said ridge having a top surface sloping away downwardly from the top surface of said ridge; said dies being arranged in pairs on each of said members with their side projections placed diametrically opposite each other pointing centerwards and the ridges running substantially in tangential direction.
4. The combination with a forging press having a stationary member and a reciprocating member; of dies adapted to be adjustably secured to said members respectively, each of said dies comprising a foot, a ridge rising from said foot and having a substantially rectangular top surface and 20 downwardly diverging side faces, and a side projection extending substantially at right angles from said ridge having a top surface sloping away downwardly from the top surface of said ridge; said dies being arranged in pairs on each of said members with their side projections placed diametrically opposite each other pointing centerwards and the ridges running substantially in tangential direction, a turntable mounted in said stationary member, means for lifting said turntable, and other means for intermittently turning said turntable a small angle between each stroke of said reciprocating member.
5. The combination with a forging press 35 having a stationary member and a reciprocating member; of dies adapted to be adjustably secured to said members respectively, each of said dies comprising a foot, a ridge rising from said foot and having a substantially rectangular top surface and downwardly diverging side faces, and a side projection extending substantially at right angles from said ridge having a top surface sloping away downwardly from the top surface of said ridge; said dies being arranged in pairs on each of said members with their side projections placed diametrically opposite each other pointing centerwards and the ridges running substantially in tangential direction, a turntable including a source of fluid pressure and conduits therefor mounted in said stationary member, means for lifting said turntable, and other means for in-
- termittently turning said turntable a small angle between each stroke of said reciprocating member and comprising a pawl and ratchet device inserted between the turntable and the stationary member.
6. A method of producing a blank of the class described, consisting in first providing a cylindrical "cheese" of correct weight and thickness; second, forming by compression tangentially running narrow channels on opposite faces of the "cheese" terminating with a sloping surface at one end of each channel running in radial direction toward the center of the "cheese", each of said channels with its corresponding sloping surface forming substantially an L-shaped contour.
7. A method of producing a blank of the class described consisting in first providing a cylindrical "cheese" of correct weight and thickness; second, forming by compression tangentially running narrow channels on opposite faces of the "cheese" terminating with a sloping surface at one end of each channel running in radial direction toward the center of the "cheese", third, turning the "cheese" a small angle; fourth, forming other channels by compression in the same manner and repeating the turning and compression alternately until the entire top and bottom surfaces have been so treated, each of said channels with its corresponding sloping surface forming substantially an L-shaped contour.
8. A die for circular forgings, comprising a foot portion adapted to be secured in a forging apparatus and a two armed body portion of substantially L-shaped configuration forming a ridge rising from the foot portion and having upwardly converging side and end surfaces, one of said arms being arranged radially and the other arm tangentially with regard to the forging, substantially as described.
9. A die for circular forgings, comprising a foot portion adapted to be adjustably secured in a forging apparatus and a ridge portion rising from the foot portion and consisting of a short arm arranged radially and a long arm tangentially with regard to the forging, and the top surface of the short arm sloping downwardly from that of the long arm in order to form a hub portion on the forging, substantially as described.

In testimony whereof we affix our signatures.

CHRISTIAN J. STEEN. [L.S.]  
EDWARD V. FINERAN. [L.S.]